

June 25, 1963

R. P. HEUER

3,094,952

RIBBED BASIC REFRACTORY ROOF

Filed May 24, 1960

2 Sheets-Sheet 1



INVENTOR  
Russell P. Heuer

BY  
Dwight L. Johnson  
ATTORNEYS

June 25, 1963

R. P. HEUER

3,094,952

RIBBED BASIC REFRACORY ROOF

Filed May 24, 1960

2 Sheets-Sheet 2



1

3,094,952

**RIBBED BASIC REFRACATORY ROOF**  
Russell Pearce Heuer, Villanova, Pa., assignor to General  
Refractories Company, a corporation of Pennsylvania  
Filed May 24, 1960, Ser. No. 31,384  
4 Claims. (Cl. 110—99)

The subject matter herein disclosed forms a continuation-in-part of the matter set forth in my co-pending application Serial No. 577,311, filed April 10, 1956, now abandoned, and the invention relates to a refractory roof comprising rib brick, intervening brick, and supplemental refractory brick superimposed on the intervening brick and the ribs.

An object of this invention is to obtain improved resistance to spalling in supplemental refractory brick in a ribbed basic furnace roof, the supplemental refractory brick suitably being installed while the furnace is operating, for the supplemental brick thereafter to endure beyond the expected life of the intervening brick in the roof and to co-function with the rib brick in the roof.

A further object is the provision of internal oxidizable ferrous plate means in the basic refractory roof brick, which plate means divides the refractory of the individual supplemental brick into a plurality of integral partitioned zones or sections which are in series with each other and with the brick in the adjacent ribs, thus for the supplemental brick to resist spalling and more reliably remain in place while being supported by the ribs of the roof.

A further object is that of providing a plurality of brick in the individual ribs, laterally of the ribs, and to have these brick in series with the refractory sections of the supplemental brick which are adapted to span the ribs while being supported by the ribs.

A still further object is the provision of external oxidizable ferrous plate means on one or more lateral outside faces of the supplemental refractory roof brick through co-molding this plate means with the refractory of the supplemental brick, and preferably introducing the internal plate means integral with the external plate means.

Other objects of the invention in part will be obvious and in part pointed out more fully hereinafter.

In the drawings I have chosen to illustrate a few only of the numerous embodiments in which my invention may appear, selecting the forms shown from the standpoints of convenience in illustration, satisfactory operation and clear demonstration of the principles involved.

FIGURE 1 is a fragmentary diagrammatic transverse section of an open hearth steel furnace of the general character employing the roof of the invention.

FIGURE 2 is a fragmentary enlarged section on the line 2—2 of FIGURE 1.

FIGURE 3 is a lateral elevation of the supplemental refractory brick of the invention, looking at the small lateral side.

FIGURE 4 is a lateral elevation of the brick of FIGURE 3, looking at the large lateral side.

FIGURE 5 is an enlarged perspective of one of the supplemental basic refractory roof brick of the invention showing one arrangement of external and internal oxidizable ferrous metallic plate means.

FIGURE 6 is a perspective view similar to FIGURE 5, showing an alternative arrangement of the plate means.

FIGURE 7 is a diagrammatic transverse vertical section showing the molding of the brick of the invention.

FIGURE 8 is a fragmentary section corresponding to FIGURE 2, but differing in the respect that the supplemental brick employed between the roof ribs are of the form represented in FIGURE 6.

2

open hearth steel furnace, comprising a hearth, not shown, framework 20 and front wall 21 and back wall 22 supported by the side framework, skewbacks 23 and 24 at the top of the front wall and back wall supported by the walls and by the framework, and a roof 25 supported partially by the skewbacks and partially by suspension from overhead framework 26.

The roof consists of rows of relatively elongated or ribbed refractory brick 27 suitably arranged in pairs as shown in FIGURE 2, and extending arcwise of the furnace to produce the ribs. Each of the ribbed brick has a hot end 28, a cold end 29, a straight lateral side 30 in the plane of the arch, a lateral side 31 and also radial sides 34. Lateral side 31 includes a straight portion 32 in the plane of the arch and a wedge or tapered portion 33 at the upper end. The rib brick are preferably basic, consisting of magnesia, chrome, chrome-magnesia or magnesia-chrome.

Interposed between the elongated or ribbed brick at the hot end are intervening rows 35 of relatively short refractory brick, which may be of wedge or key construction as desired, and have hot ends 36, flat archwise surfaces 37, radial surfaces 38 and cold ends 40. The intervening brick are preferably basic, consisting of magnesia, chrome, chrome-magnesia or magnesia-chrome.

The relatively elongated brick 27 are desirably independently supported from overhead structure in any desired manner in the form shown. Arcuate metallic beams 41 carried by suspension elements 42 from the overhead structure 26 conform to the cold ends of the ribbed brick. Holes 43 across the ribbed brick near the cold ends receive metallic hangers 44 which are suitably bands of wire extending around the beams 41 and twisted at 45.

The intervening relatively short brick 35 are desirably sprung from the skewbacks 23, 24 at the front and back of the furnace.

The use of dot and dash lines in FIGURE 2 suggests destruction at the hot ends of the brick to form a hot end line 46 after the brick have been in service for some time.

One of the advantages of the structure of FIGURES 1 and 2 is that the intervening brick 35 can be backed up by supplemental brick 47 at the cold end after the roof is partially consumed, as shown in FIGURE 2. These supplemental brick greatly increase the life of the roof.

It is customary practice in operating such a roof to allow the roof to burn away as shown in FIGURE 2 to some level 46 at which it becomes necessary to place supplemental brick which will be held in position by the ribbed brick. This operation of placing the supplemental brick can be performed while the furnace is operating at high temperature.

As the roof continues to wear away the intervening brick 35 below the supplemental brick are completely eliminated and the supplemental brick are exposed to the flame of the furnace. Due to the character of the construction, the exposed hot faces of the supplemental brick are large, being perhaps twelve inches long by two and one-half inches wide.

I have found that these brick having such a large working face tend to spall very rapidly. It is not possible to make the exposed faces of these brick smaller because they have to be long enough to reach between the successive rib brick of the roof.

I have discovered, however, that the spalling above referred to is greatly reduced if the supplemental brick are molded of a basic refractory composition consisting of magnesia, or mixtures of magnesia with alumina and/or chromite, and where the amount of magnesia present is 10 percent or more by weight of the refractory composition. Then by comolding this composition with internal oxidizable ferrous metal plate means which extends be-

FIGURES 1 and 2 illustrate a furnace, suitably an

tween the hot face and cold face of the supplemental brick and subdivides the refractory into a plurality of partitioned sections or zones integrally in series with each other and the plate means, the partitioned brick behaves as if a number of small brick were present, thus greatly increasing the resistance to spalling. At the same time the brick functions as a large brick from the standpoint of support between the ribs and therefore the various partitioned sections introduce no problem in the sense of needing additional support in the roof. The internal oxidizable ferrous plate means also contributes a strengthening function in the brick through being in intimate contact with the magnesia in the refractory composition and through effects which the operating conditions of the furnace have upon the plate means and the refractory when the supplemental brick are exposed to the flame of the furnace. Strengthening zones of magnesioferrite develop in the brick by virtue of the ferrous substance of the plate means and the adjacent magnesia in the brick being altered to magnesioferrite which then stands as a barrier against spalling and cracking at the hot face of the supplemental brick. The overall pattern of spalling and cracking which one might normally expect is very appreciably altered by the internal plate means and by the magnesioferrite barriers which ultimately occur in the brick as the result of its use in the furnace. The supplemental brick accordingly are well equipped to share long life in the roof with the rib brick which still remain to afford support and to contribute their refractoriness in the roof. Usually, the rib brick, the intervening brick, and the supplemental brick all are made having substantially the same basic refractory composition for the sake of uniformity although in certain instances these basic refractory compositions may differ depending for example upon specific needs.

It is also very desirable to provide lateral surface plates of oxidizable ferrous metal on the supplemental brick.

The method of molding is illustrated by FIGURE 7 which shows a molding press 48 comprising relatively movable upper and lower dies 50 and 51 and mold sides 52 forming a mold cavity 53 which is desirably of wedge or tapered contour in plan view.

Before filling the mold with refractory, a lateral surface plate 54 is desirably placed on the bottom die, and preferably secured to the surface plate and extending upwardly in a generally longitudinal direction are internal plates 55, also tabs 56 lanced out from the surface plate extend upwardly to engage in the refractory. The lancing of the tabs leaves openings 57 in the surface plate, as best seen in FIGURE 5.

The mold is filled with a loose refractory mass 58 as later explained. On the bottom of the top die 50 is placed a cooperative and suitably identical surface plate 54 having secured thereon downwardly protruding internal plates 55 and downwardly protruding tabs 56. The internal plates 55 from the top plate combination desirably are aligned with the similar internal plates from the bottom plate combination. The upper plate combination is suitably held on the upper die by a magnetic chuck, a mechanical gripper or by an adhesive, as desired, during the molding.

When the upper and lower dies move relatively together, the internal plates are buried in the refractory brick by comolding and the tabs are similarly buried while the surface plates are united to the brick by comolding through the internal plates and the tabs.

In the final brick as shown in FIGURE 5, the internal plates are suitably slightly diverging but generally transverse to the hot face 58 of the brick. The internal plates are close together but preferably do not meet at 60 near the center. The internal plates desirably extend substantially the entire distance from the hot face 58 to the cold face 61, although considerable advantage will be obtained from the invention if, beginning at about the hot face of the brick, they extend more than 75 percent of the distance

to the cold face and excellent results can be obtained if the internal plates extend 85 percent of this same distance.

In the form shown, the arcwise faces 62 of the brick are slightly wedge-shaped to conform to the arch and carry the external plates 54. The radial side surfaces 63 are pronouncedly wedge-shaped and engage against the wedge surfaces 33 to support the supplemental brick from the rib brick. The internal plates divide the refractory of the brick into four partitioned sections which are in series laterally of the ribs of the roof (see FIGURE 2) and the sections also are in series with the rib brick widthwise of the adjacent ribs. By having a plurality of rib brick widthwise of the ribs these individual brick have an influence on the pattern of cracking and spalling of the roof and the influence is shared with the partitioned sections of the supplemental brick.

The metal used for the external and internal plates is preferably steel or iron, including plain carbon steel, alloy steel or stainless steel. The plates are all sheet material, preferably having a thickness of approximately between  $\frac{1}{32}$  inch and  $\frac{1}{4}$  inch, depending upon the installation.

In the preferred embodiment as shown, the surface plate 54 is desirably connected as by welding to the internal plate or plates 55 which extend transversely from the surface plate preferably in line with the internal plate extending from the opposite side. Thus the internal plates, in the installed positions of the supplemental brick, are disposed generally arcwise of the roof and are between the corresponding pair of adjacent ribs of the roof. The partitioned sections in the supplemental brick may suitably lie in arcwise rows extending from the front to the back of the furnace and which occupy positions between the ribs and advantageously occur with plural arcwise rows of the rib brick in each of the individual ribs and so that the hot face of the roof is continuously formed having small areas of basic refractory which at least to some extent are isolated one from the other against carry-over of cracking and spalling.

The surface plates may if desired be of U-shaped formation to provide external plates at the radial sides. In order to accomplish the molding with a U-shaped plate, the U-shaped plate is placed in the bottom of the mold and the loose refractory is placed on it and inside it. The upper plate is placed on the upper die and then the dies are brought together.

The number of internal plates to be used, whether one or several in a particular brick, will depend upon the overall length of the supplemental brick or the distance between ribs. In the simplest form it is sufficient to use only one internal plate which may divide the brick into two approximately equal parts. In other cases two, three, or even four or more internal plates preferably spaced at equal distances from each other and from the radial side of the brick will provide suitable arrangements.

The internal plates should be at right angles to the external plate in order to lie in the direction of the motion of the pressing die. The plane of the internal plates may also if desired be perpendicular to the internal surface of the roof although slight inclination is proper, as shown in FIGURE 5, so that the internal plate nearest the radial side of the brick is almost parallel with the radial side.

The internal plates oxidize in service and the iron oxide formed by the oxidation of the internal plates reacts with the magnesia in the basic refractory to form magnesioferrite which partly diffuses into the refractory and causes no appreciable volume expansion.

Thus the oxidizable internal plates partition the brick into two or more parts, each of which behaves as if it were a small individual brick. On the other hand, the supplemental brick is supported as a unit, but the spalling behavior is that characteristic of the small component parts.

The oxidizable iron or steel plates exert a pronounced tendency to prevent spalling off of the hot ends of the brick. The magnesioferrite which forms in the vicinity

of the plates near the hot ends is highly refractory and tends to create a strengthening plane running transverse to the span of the brick between the adjacent ribs.

The planar distribution breaks up the forces which cause cracking and thus tends to prevent crack propagation across the brick from one side of the magnesioferrite to the other. Thus spalling off at the hot end is prevented or retarded. The tapered ends of the supplemental brick which rest upon the suspended ribs are less prone to severe cracking and spalling since the carry-over of severe cracks is arrested by the magnesioferrite.

Any suitable basic refractory containing magnesia as above described capable of use without kiln firing may be employed. A low temperature binder will desirably be used such as sulfuric acid or an organic binder. After molding the brick are cured and/or dried and are then ready for use. The external plates on the brick where used tend to protect the brick against damage during shipment. The supplemental roof brick are usually installed in the unfired condition and are fired through furnace operation, at which time the magnesioferrite is formed.

While the illustration in FIGURE 1 shows an arc structure, it will be understood that the roof may be flat if desired.

While I have shown the internal plates attached to the external plates, it will be understood that the internal plates may be separate and may be used even without external plates.

FIGURE 6 shows a supplemental brick having internal plates 55' provided with tabs 56' on both surfaces united by comolding to the brick. There are also external plates 54' optionally used and having internal tabs engaging in the refractory and held by comolding.

In this case the internal plates lie in a plane generally parallel to the pressing dies. In manufacturing these brick the bottom plate 54 is first inserted with its tabs sticking up. Then a layer of loose refractory which forms the refractory portion 64 is inserted, after which an internal plate 55' is put in having tabs extending upwardly and tabs extending downwardly. Then the loose refractory forming the brick portion 65 is inserted and another internal plate 55' follows. Then the loose refractory forming the brick portion 66 is inserted and finally the external plate 54' is placed on the top die. In this form the internal plates are shown extending to the radial edges, but it will be evident that they can extend only partially to such edges if desired. The comolding and the tabs unite the refractory and the plates together into a unitary structure. The resulting supplemental brick 54' in this instance individually have a plurality of partitioned sections which are in series with each other and the oxidizable ferrous plates with the partitioned sections or zones of the basic refractory, of the type hereinbefore referred to containing at least about 10 percent magnesia, are in series which extends arcwise of the roof when brick 54' are substituted for the supplemental brick 54 in the manner indicated in FIGURE 8. Further, in this particular use, each partitioned section in the supplemental brick occurs in series with the rib brick in the adjacent ribs, transversely of the ribs. Cracking and spalling again are effectively arrested in the hot face pattern of the roof which includes the refractory sections of the supplemental brick 54' and the hot faces of the rib brick. The magnesioferrite which forms from the oxidizable internal ferrous plates 55' and the magnesia present adjacent to these plates not only produces crack barriers but strengthening zones so that the supplemental brick serve quite well as the short beams which they are, spanning the gap between the adjacent roof ribs on which the supplemental brick rest. In being formed, the magnesioferrite brings about no appreciable increase in volume and thus stresses in the roof are minimized.

In view of my invention and disclosure, variations and modifications to meet individual whim or particular need will doubtless become evident to others skilled in the art, to obtain all or part of the benefits of my invention without copying the product shown, and I, therefore, claim all such insofar as they fall within the reasonable spirit and scope of my claims.

Having thus described my invention, what I claim as new and desire to secure by Letters Patent is:

1. A furnace roof for use on a metallurgical furnace, comprising skewbacks on opposite sides of the roof, metallic supporting structure running across the roof from one skewback to another above the level of the roof, a plurality of spaced rows of basic refractory longer brick 10 extending as ribs between the skewbacks, each of said basic refractory longer brick having cold ends and hot ends, being laterally tapered adjacent the cold ends and having lateral parallel side portions adjacent the hot ends, each of said basic refractory longer brick extending generally vertically from the hot surface of the roof through the thickness of the roof to the cold end, metallic hanger support means interconnecting said longer brick at the cold ends with said supporting structure, said longer brick being supported by said hanger support means, intervening basic refractory brick positioned between said longer rib brick having a shorter length than the rib brick and extending upward from the hot surface of the roof along the lateral parallel portions of the rib brick, said intervening basic refractory brick having lateral parallel sides 15 adjoining the lateral parallel side portions of said rib longer brick and said intervening basic refractory brick being in plural arch rows between the adjacent ribs and supported by said skewbacks, independently of said rib brick, and supplemental basic refractory brick containing magnesia in amounts of 10 percent or more in the refractory composition thereof and being superimposed as short beams between said longer rib brick above said intervening brick and extending laterally across said plural arch rows of said intervening brick, said supplemental basic 20 refractory brick having oxidizable ferrous metal plates internally thereof dividing the magnesia-containing refractory composition thereof into a plurality of partitioned sections each extending at least a major portion of the distance between the corresponding hot faces and cold faces of said supplemental brick and extending in the direction toward and away from the skewbacks, each of said supplemental brick having lateral tapering sides which engage the laterally tapering sides of said rib brick and being supported by said rib brick and thus placing said 25 partitioned sections in series laterally with rib brick in the adjacent ribs.

2. A furnace roof of claim 1, in which said supplemental brick have external oxidizable metallic plates on radial faces thereof, extending from one lateral tapering side to the other.

3. A furnace roof of claim 1, in which said partitioned sections in individual ones of said supplemental brick are in series with each other laterally of the adjacent ribs.

4. A furnace roof of claim 1, in which said partitioned sections in individual ones of said supplemental brick are in series with each other arcwise of the roof.

#### References Cited in the file of this patent

#### UNITED STATES PATENTS

- |    |           |                    |                |
|----|-----------|--------------------|----------------|
| 65 | 2,652,793 | Heuer et al. ----- | Sept. 22, 1953 |
|    | 2,824,529 | Ries -----         | Feb. 25, 1958  |
|    | 2,903,254 | Heuer -----        | Sept. 8, 1959  |

#### OTHER REFERENCES

- 70 Heuer, R. P. and Fay, M. A.: "The All-Basic Open Hearth European and American," Journal of Metals, pages 824-829, June 1950.